

# UNITED STATES PATENT OFFICE.

ACHILLES DE KHOTINSKY, OF GELNHAUSEN, PRUSSIA, GERMANY.

## MANUFACTURE OF CARBON FILAMENTS.

SPECIFICATION forming part of Letters Patent No. 429,535, dated June 3, 1890.

Application filed February 3, 1890. Serial No. 339,082. (No model.)

*To all whom it may concern:*

Be it known that I, ACHILLES DE KHOTINSKY, a subject of the Emperor of Russia, residing at Gelnhausen, Kingdom of Prussia, 5 Germany, have invented new and useful Improvements in the Manufacture of Carbon Conductors for Electric Incandescent Lamps, whereof the following is a specification.

The subject of my invention consists in a 10 process for rendering natural cellulose entirely void of structural constitution and for producing therefrom carbon conductors for electric incandescent lamps, which are superior to those heretofore made from cellulose. 15 For this purpose I employ threads of purified natural cellulose—preferably such as are made from cotton—which has been freed from fatty matter and treated with muriatic or hydro-fluoric acid, or both, in view of extracting all 20 mineral substances. These threads are steeped at the ordinary temperature in phosphoric acid having a specific gravity of about 1.70 and left therein about one minute. After having been taken out of the acid they are 25 hung up in air which is as dry as possible, so that the phosphoric acid imbibed by the thread may not become diluted by attraction of moisture. The acid which is in excess drips off, while the portion remaining in the 30 thread converts the same by acting progressively from the exterior to the interior into a translucent mass. For this conversion about twenty-four hours are required, so that its progress may conveniently be watched. The 35 threads in which the structural constitution has entirely disappeared are withdrawn from the further action of the acid by dipping them into a liquid adapted to separate phosphoric acid from the cellulose, such as alcohol, ether, and distilled water. Preferably a 40 mixture of two volumes of ethyl ether and one volume of ethyl alcohol are employed. The phosphoric acid, being heavier than the said liquids, runs off and the thread finally presents itself as a white amorphous mass. The 45 threads are thereupon washed with distilled

water until every trace of acid has been removed and dried. In view of making their surface smoother and their thickness more uniform they may then be passed through a 50 draw-plate. Finally the threads are carbonized in known manner, and the conductors thus obtained are employed in incandescent lamps, as usual.

I am aware that threads of natural fibrous cellulose have heretofore been treated with sulphuric acid in view of converting them into a structureless mass of gelatinous cellulose. The sulphuric acid, however, acts so rapidly on the fibrous cellulose that it is impossible to properly control the process, many threads becoming completely destroyed, while others are only superficially acted upon; but if phosphoric acid of the prescribed degree of concentration is employed at the ordinary 60 temperature of the air the conversion of the fibers into gelatinous cellulose goes on slowly, so that its progress may be accurately watched. The described process, therefore, presents the advantage of affording means for easily obtaining threads of uniform quality. 70

I claim as my invention—

The process of producing carbon conductors for electric incandescent lamps, which consists in impregnating threads of purified 75 natural cellulose at the ordinary temperature with phosphoric acid having a specific gravity of about 1.70, in leaving the same to the action of the acid in dry air until their structural constitution has disappeared, in removing the phosphoric acid by treatment with a liquid adapted to separate out said acid—such as alcohol, ether, and distilled water—and in carbonizing the amorphous thread, substantially as described. 80

In testimony whereof I have hereunto set my hand in the presence of two subscribing witnesses.

ACHILLES DE KHOTINSKY.

Witnesses:

JEAN GRUND,  
ALVESTO P. HOGUE.